

Patented Aug. 28, 1923.

1,466,380

# UNITED STATES PATENT OFFICE.

HARRY NUSBAUM AND JOSEPH NUSBAUM, OF PHILADELPHIA, PENNSYLVANIA,  
ASSIGNORS TO P. E. SHARPLESS COMPANY, OF PHILADELPHIA, PENNSYLVANIA,  
A CORPORATION OF PENNSYLVANIA.

## PROCESS OF COATING METAL FOIL WITH PARAFFIN, AND THE PRODUCT THEREOF.

No Drawing.

Application filed March 31, 1921. Serial No. 548,537.

To all whom it may concern:

Be it known that we, HARRY NUSBAUM and JOSEPH NUSBAUM, citizens of the United States, residing at the city of Philadelphia, 5 in the county of Philadelphia and State of Pennsylvania, have jointly invented a certain new and useful Improvement in Processes of Coating Metal Foil with Paraffin and the Product Thereof, of which the following is a specification.

Our invention relates primarily to a new method and means hereinafter described for fixedly applying a coating of paraffin, commonly called paraffin wax, to the 10 surface of metal foils, such as tin foil or aluminum foil commonly employed, for sanitary and other reasons hereinafter mentioned, as a wrapper for those articles of food, such for example as soft cheese, which require 15 for commercial purposes, to be enclosed in a suitable wrapping material; but the ultimate object, of our invention is the new product resulting from the process, which is such a metal foil so coated and hence particularly well adapted as a wrapper for 20 such perishable articles, the composition coating being odorless and operating as a preservative of the wrapped contents from the destructive or deteriorating effect of air 25 and moisture and other extraneous influences, and incidentally for sanitary reasons, and, because the composition produces a thin and transparent coating it can be advantageously used where the foil wrapper 30 has previously had a label printed directly thereon. The novelty in the process and the resultant product, resides in the fact that the composition is of such character and has such properties, as hereinafter 35 stated, that it will attach itself, with tenaciously clinging effect, to the surface of the metal foil.

We are aware it was long well known in the art to coat the surface of paper, cloth 45 and the like, with a melted composition of such paraffin wax, or with beeswax as a substitute, and sometimes with the addition to either or both, of resin, but in such disproportionate quantity as to make it objectionable for several reasons. However the 50 application of a paraffin coating to metal foil presented a very different problem from that of its application to paper or the like; and in a Patent No. 1399270 granted to one

of us, Joseph Nusbaum, is described the discovery that when proportionately small percentages of pure beeswax and purified resin, say 15 parts, in the aggregate, are combined under melting heat with a very large proportion of paraffin wax, such as about 85 60 parts of the latter, the purified resin and pure beeswax, will apparently combine with the paraffin wax and cause it to attach itself fixedly to the skin surface of the foil to the extent at least, of not peeling or cracking under flexure from ordinary handling, and moreover produces a thin, odorless, colorless and hence transparent coating thereon. While this composition 65 fully performed the functions for which it 70 was used, we found in it some lack of pliability or excess of brittleness and some tendency to undue adhesiveness tending to tear the foil in handling it, which seemed to indicate the necessity for a solvent of the 75 resin, as a constituent in the composition, and suggested to us to try a mineral oil for this purpose, not inconsistent with the paraffin as a petroleum product, because we had learned, from a previous Patent No. 1194340 80 for a different composition and purpose, that such had been used as a solvent of vegetable wax and gum; and also that it might otherwise operate beneficially on the other elements of our patented composition and 85 produce the improved results we sought for; and our experiments immediately made therewith or those then made under our direction, demonstrated satisfactorily to us that the use of such a mineral oil in our 90 composition, as such solvent and combining agent was desirable and very effective to 95 overcome both the objections stated.

Our present invention is predicated on that theory and is an improvement on our 95 composition of that patent, or rather a substitute therefor, in which, while the relative proportion of the base—paraffin wax—remains the same, the relative percentage of beeswax and resin are reduced, and a mineral oil solvent, which, like the paraffin, is 100 a derivative of petroleum, substituted to the extent to which the resin and beeswax are reduced.

To these ends the novelty of our present 105 process and product, consists primarily in the discovery that a paraffin wax coating can be caused to fixedly adhere to the skin sur-

face of metal foil by admixing with it, in the melting pot, certain combining elements of the character hereinabove mentioned and substantially in the proportions hereinafter stated; and secondly in increasing the fluidity of the composition by raising its temperature some ten or twenty degrees C. above the melting point of its least meltable constituent and so maintaining it during the application of the composition to the surface of the foil.

In the practice of our invention we use commercial tin foil or aluminum foil, of a suitable thickness for the purpose for which it is to be ultimately used; and then make up a coating composition therefor consisting of the following elements, in substantially the relative proportions, stated in percentages of weight, as follows: Paraffin wax, 87.5 per cent; pure beeswax 5 per cent; purified resin 4 per cent, and mineral oil derived from petroleum 3.5 per cent.

The ingredients named in the relative proportions stated are mixed in a steam-jacketed kettle, preferably, in which they combine in a melted mass at about 100° C. to form a homogeneous mixture and of free fluidity; the mineral oil being preferably added in very small divided quantities at intervals during the time required for the melting of the other elements. A slight increase of temperature, say 10 to 20 degrees F. above that stated for melting, will increase the fluidity and its heat, and is for those reasons desirable when applying the composition as a coating on metal foil.

Our new composition has, as its base, a pure paraffin sometimes called paraffin wax, which is a colorless or white solid, more or less translucent, odorless, tasteless, and slightly greasy to the touch. It is a well known commercial product, and is said to be a purified mixture of solid hydrocarbons commonly obtained from petroleum. That which we use and buy in the open market, has a melting point of about 52° C. It should form 85% to 87% by weight, of the total weight of our new composition.

The beeswax used in this composition should, to obtain the best results in all the respects stated, be entirely free from impurities, in other words the pure beeswax unadulterated, which is of a light lemon color and has a melting point of about 65° C. or 150° F., or very nearly the same as pure paraffin wax. It has the property of readily uniting with paraffin wax and purified resin.

The resin used should, for like reasons, be free from impurities, hence if ordinary commercial resin be used, it should be enclosed in a textile bag during the melting with the other elements of the composition, whereby the non-soluble or foreign matters, usual in such resins, will be conveniently separated

out in the melting process. A very pure resin, of a character particularly compatible with the mineral oil, and which we have used with good results, is a product of the Barrett Chemical Co., readily obtained in the open market, and is commercially sold under the trade name "Cumar" which, perhaps, is an abbreviated derivation of its technical descriptive name "Paracoumarone." It is of the usual resin color, one grade of which is light brown, in color, which softens at about 70° C. and melts at 90-100° C.

We combine with these elements, preferably after bringing them into a melted and mixed state, (the resin constituent being the least meltable of them,) a small percentage of mineral oil, which, like the paraffin base, is also a derivative of petroleum, and is equally colorless, transparent, odorless and tasteless. A suitable example of it which we have used with the best results, is that made and sold commercially by the Standard Oil Co. of New Jersey, under the trade name "Acto". The mineral oil is employed as a solvent of the resin and also for its probable toughening effect on the beeswax; and it apparently operates also to unite with them and the paraffin base in producing a homogeneous mixture. As the result of our repeated experiments and commercial use of it, we found that it entirely overcame the objectionable tendencies of the resin constituent in our previous composition, and produced a composition which gives a thin, transparent, and extremely pliable coating; these resultant effects being markedly apparent.

The new composition is in liquid form, of a dark brown, at the melting temperature which will produce a combining fluidity of all its components, which is about 100° C. When raised in temperature to say 120° C. to increase its fluidity and impart a high temperature to it, a very thin and evenly distributed coating can be had by a quick dipping, by suitable means, of the foil wrapper to be coated; a thin coating being less brittle and more pliable, and moreover more transparent, hence if applied to a metal foil having printing on it, will permit the printing thereon to be easily read through it. It sets or dries very promptly; will resist peeling or cracking when flexed under ordinary conditions of usage; is free from any odor, and, to the extent to which the coated wrapping is so applied as to exclude air from its contents, will, for that reason, prevent the growth of aerobic molds on any food product thus brought into enclosing contact with it.

Having thus described our invention, we claim:

1. The process of causing a coating of paraffin wax to fixedly adhere to the surface of metal foil, such as tin foil or aluminum

foil, which consists in combining with the paraffin wax, in a suitable vessel, under applied heat, purified resin, beeswax and a mineral oil derived from petroleum, in substantially the proportions specified, and maintaining the melting temperature and fluidity of the composition during the application thereof to the foil to be coated.

2. The process of producing and causing to fixedly adhere to the surface of metal foil an odorless, transparent, and moisture and air-resisting coating, which consists in forming a compound in a suitable vessel, under applied melting heat, consisting of paraffin wax, a mineral oil derived from petroleum, purified resin, and natural beeswax, in substantially the proportions specified; then raising the temperature about 10 to 20° C. to increase the fluidity of the composition, and dipping therein the foil to be coated.

3. The new product described which is a metal foil coated with a composition consisting of paraffin wax, beeswax, purified resin, and a mineral oil, in substantially the proportions specified, and capable of flexure without substantially disturbing the fixed adherence of the coating to the foil.

4. The new product described which is a metal foil, such as tin or aluminum foil, having on its surface an odorless, thin and transparent coating produced by the application thereto of a composition consisting of paraffin wax, beeswax, purified resin and a mineral oil derived from petroleum, compounded in substantially the proportions specified.

5. The new product described which is a preservative wrapper for a perishable article, consisting of a metal foil, such as tin foil or aluminum foil, having on the surface thereof a moisture and air-proof coating formed by the application thereto, in a fluid and heated state, of a composition of paraffin wax, beeswax, purified resin and mineral oil, in substantially the proportions specified.

In testimony whereof, we have hereunto affixed our signatures this 28th day of March 1922.

HARRY NUSBAUM.  
JOSEPH NUSBAUM.

Witnesses:

I. M. TUNIS,  
HARRY A. GREAR.